

# UNITED STATES PATENT OFFICE.

JULIUS Q. GILL, OF PEORIA, ILLINOIS.

## COOLING COMPOUND FOR HOT JOURNAL BOXES AND PROCESS FOR PRODUCING THE SAME.

1,428,103.

Specification of Letters Patent. Patented July 18, 1922.

No Drawing.

Application filed August 2, 1920. Serial No. 400,634.

To all whom it may concern:

Be it known that I, JULIUS Q. GILL, a citizen of the United States, residing at Peoria, in the county of Peoria and State 5 of Illinois, have invented new and useful Improvements in Cooling Compounds for Hot Journal Boxes and Processes for Producing the Same, of which the following is a specification.

10 The invention relates to a cooling compound for hot boxes, and process for producing the same.

15 The object of the invention is the production of a compound designed for cooling hot boxes on railways and street cars, locomotives and in fact any vehicle in which that condition occurs, and adapted when mixed with a heated lubricant of reducing the temperature of the moving parts.

20 The compound is designed for use in emergency for cooling a hot box and is adapted to be readily applied to the same without removing the heated lubricant from the journal box.

25 This compound consists of a mixture of vegetable oils, such as corn oil and castor oil, alkali such as caustic soda, soda ash and potash, carbon such as ivory black, methyl salicylate, free alkali as carbonates and 30 moisture. The ingredients of the cooling compound are preferably mixed in the following proportions:

|                           | %      |
|---------------------------|--------|
| Corn oil                  | 35.59  |
| Castor oil                | .89    |
| Alkali                    | 6.826  |
| Ivory black               | .534   |
| Methyl salicylate         | .89    |
| Free alkali as carbonates | .36    |
| 40 Moisture               | 55.00  |
| Total                     | 100.00 |

In preparing the cooling compound, a 45 kettle is charged with 100 lbs. of corn oil to which is added 50 lbs. of water. Heat is then applied and the contents thereof are then warmed to approximately 120° F. Then add 25 lbs. of caustic soda solution at 50 35 degrees Baumé and bring the contents to a boil and continue at a gentle boil until it thickens up and shows dry on a spatula. Then add to the mixture 5 lbs. of soda ash dissolved in 25 lbs. of water and then run 55 in 25 lbs. of potash solution at 40 degrees

Baumé. Now boil thoroughly until the mass has settled low in the kettle and shows up clear and transparent on the spatula. Now to finish up and fit with alkaline strength, take samples on the spatula, allow 60 them to cool off and test with a drop of phenolphthalein 5% solution. If the mixture fails to react red, add a very small amount of potash at 40 degrees Baumé and boil thoroughly and test again. Continue 65 this operation until a faint red reaction from the phenolphthalein takes place. 40 lbs. of water are then added in order to bring the yield of compound up to 2½ lbs. to the 70 pound of oil.

During the boiling operation, a portion of the moisture will have been evaporated and this is compensated for by adding at the finish 1½ lbs. of ivory black mixed with a small quantity of hot water, 2½ lbs. of 75 methyl salicylate and 2½ lbs. of commercial castor oil. The contents of the kettle are then thoroughly stirred and a finish test made with phenolphthalein. If this last test fails to show a red reaction because of the 80 castor oil having taken up all the free alkali, the mass should be once more treated with a small portion of potash solution until it shows a faint red reaction at which time the heat may be shut off and the material drawn 85 off for shipment.

What is claimed is:—

1. A cooling compound for hot boxes, which consists of corn oil, castor oil and caustic alkali in such proportion as to form 90 soap, a small amount of free alkali, ivory black, methyl salicylate, and water in such proportion as to constitute more than 50% of the mixture.

2. A cooling compound for hot boxes, 95 which consists of soap consisting of 35.59% corn oil, .89% castor oil and 6.826% caustic alkali; .534% ivory black, .89% methyl salicylate, .36% free potash, and 55% water.

3. The process of cooling hot boxes, which 100 consists in applying thereto a cooling compound, the constituent ingredients of which are corn oil and castor oil soaps, free alkali; ivory black, methyl salicylate, and a large proportion of water.

4. The process of cooling hot boxes, which 105 consists in applying thereto a cooling compound, the constituent ingredients of which are soap consisting of 35.59% corn oil, .89% castor oil and 6.826% caustic alkali; .534% 110

ivory black, .89% methyl salicylate, .36% free potash and 55% water.

5. The herein described process for producing a cooling compound for hot boxes and the like, which consists in boiling corn oil and caustic soda and then adding soda ash and water and continuing the boiling

operation and then adding ivory black, methyl salicylate and castor oil and finally adding enough potash to give a faint red re- 10 action with phenolphthalein.

In testimony whereof I have hereunto affixed my signature.

JULIUS Q. GILL.